

June 26, 1923.

1,460,049

W. B. BALLANTINE

WORKABLE METAL ARTICLE

Filed March 29, 1921

*Fig. 1.*



*Fig. 2.*



INVENTOR

William Bonner Ballantine,  
Bynes, Stetini, Burgess, Carmely,  
his Atts.

## UNITED STATES PATENT OFFICE.

WILLIAM BOWMAN BALLANTINE, OF LONDON, ENGLAND.

## WORKABLE METAL ARTICLE.

Application filed March 29, 1921. Serial No. 456,750.

(GRANTED UNDER THE PROVISIONS OF THE ACT OF MARCH 3, 1921, 41 STAT. L., 1313.)

*To all whom it may concern:*

Be it known that I, WILLIAM BOWMAN BALLANTINE, a subject of the King of England, residing in London, England, have 5 invented certain new and useful Improvements in Workable Metal Articles (for which I have filed an application in Great Britain Oct. 29, 1919, Ser. No. 158,329), of which the following is a specification.

10 This invention lies in improvements in or relating to the production of rustless articles of steel. At present such articles are produced from a steel alloy containing a proportion of chromium, generally with nickel 15 or other element in addition, and this alloy is in itself expensive.

The object of this invention is to diminish the cost of articles which possess a surface which is rustless or noncorrodible.

20 According to this invention, in the production of a rustless or non-corrodible article, a core of a steel not in itself non-corrodible, and at a suitably high temperature, is encased in a rustless layer by casting a 25 previously prepared alloy of non-corrodible or rustless chrome steel around said hot core.

In the accompanying drawings there are 30 illustrated certain embodiments of the present invention, it being understood, however, that the drawings do not define the limits of this invention, as changes may be made in the constructions therein disclosed without departing from the spirit of the invention or scope of my broader claims.

35 In the drawings,—

Figure 1 is a perspective view illustrating one embodiment of the present invention; and

40 Figure 2 is a similar view illustrating a modified form of article produced in accordance with the present invention.

45 Thus, according to one embodiment of this invention, where it is desired to produce steel bodies capable of being worked, as by rolling, drawing or forging, a core 2 of any suitable shape is formed of an ingot of ordinary steel, and around this ingot, at the required temperature, there is cast an alloy 1 of non-corrodible or rustless steel, in such a 50 way that a homogeneous junction is made between the internal core and the outer covering of rustless steel.

In one method of carrying this invention into effect, an ingot of ordinary steel is placed in an ingot mould, of internal diameter larger than the diameter of the ingot, so as to leave an annular space between them. This annular space is filled up with the molten non-corrodible steel while the ingot is hot. An article produced in this manner 60 is illustrated in Figure 1 of the drawings.

Again, in the case where it is desired to produce tubes, the internal and external surfaces of which are rustless, a hollow cylindrical ingot 2' of ordinary steel may be employed, having a central pin or core and an outer ingot mould, both of which are separated from the hollow steel ingot so as to leave annular spaces outside and inside the hollow ingot, and while the ingot is hot the 70 annular spaces are filled with the molten chrome steel alloy 1', as shown in Figure 2.

In the previous application No. 1,145,925, (Sulman and Anr.) (No. 11688 of 1919), there is described a process for the production of ferro-alloys for castings, resistant to rust and corrosion, by reducing a chemical compound (for example of oxides) of iron and chromium with a thermo-reducing agent, and by introducing silicon into the 80 alloy by the employment of silicon-containing material in the thermo-reduction mixture.

Where it is desired to produce steel bodies which do not require to be rolled, drawn or forged, it is within this invention to employ a core (say of cast steel), and to cast around it a ferro-alloy containing chromium and silicon, so as to produce an article which can be machined and polished, which will have a 90 rustless and non-corrodible surface, and the core of which possesses the properties of the steel employed therein.

It will be understood that the composition of the core, and the shape of the core and 95 covering, at the time of casting, may be varied without departing from this invention.

What I claim as my invention and desire to secure by Letters Patent is:—

1. A workable metal article comprising a core of corrodible ferrous material having a non-corrodible ferro-alloy united thereto to render said article non-corrodible and permit working thereof.

2  
2. A workable metal article comprising a tubular core of corrodible ferrous material having a non-corrodible ferro-alloy united thereto on both sides thereof, to render said article non-corrodible and permit working thereof.

In testimony whereof I have signed my

name to this specification in the presence of two subscribing witnesses.

WILLIAM BOWMAN BALLANTINE.

Witnesses:

GRAHAM C. McHARDY,

AGNES E. MILLS.